

## UNITED STATES PATENT OFFICE

2,346,156

## COMPOUNDED LUBRICANT

Bruce B. Farrington, Victor M. Kostainsek, and  
George H. Denison, Jr., Berkeley, Calif., assign-  
ors to Standard Oil Company of California, San  
Francisco, Calif., a corporation of Delaware

No Drawing. Application February 16, 1942,  
Serial No. 431,116

19 Claims. (Cl. 252—32)

This invention relates to a new and useful composition of matter. More particularly, the invention involves liquid lubricating compositions for use in internal combustion engines of modern design using hard metal bearings which are susceptible to corrosion by highly refined lubricants under severe operating conditions. The invention provides a novel corrosion inhibited oil capable of inhibiting deleterious corrosive and other effects under the higher bearing pressures, the higher rotating speeds, the higher engine temperatures and the like, caused by relatively recent changes in engine design. The prevention of undue corrosion by lubricants encountering these conditions is increasingly difficult for three principal reasons.

The first reason is that the newer bearing metals are, in general, more susceptible to the destructive agents of a corrosive nature even though these metals are harder and capable of carrying higher loads than were the conventional Babbitt bearings. Typical of these corrosion-susceptible newer bearings are those composed of cadmium-silver or copper-lead alloys supported upon a steel back. Others of these relatively new bearing metals are cadmium-nickel alloys and the so-called high lead bearings.

The second reason for increasing difficulty in preventing corrosion is that the changes in engine design have required concurrent marked advances in methods of refining lubricating oils to yield products having high viscosity index or other desired properties. This demand for oils having lesser change in viscosity with changes in temperature, i. e. higher viscosity index, has been met by refining lubricants by certain selective solvent refining or selective solvent extraction processes wherein the lower viscosity index hydrocarbons are selectively dissolved. The selective solvent refining processes are operated to concentrate in one fraction, usually the undissolved lubricant fraction, those compounds of a "paraffinic" nature which show a smaller change in viscosity upon change in temperature. Selective solvent extraction processes have been found in many cases to yield an oil which, although satisfactory from the standpoint of viscosity index, is over-refined as respects stability at higher temperatures. This is particularly true where the selective solvent refinement is carried to a point which yields high viscosity index products.

By "over-refined" oils it is intended to designate those oils from which naturally-occurring inhibitors normally present in the oil have been removed at least to an extent which materially reduces the stability of the oil against deterioration at higher temperatures or which substantially increases corrosiveness of the oil on modern bearing metals. Over-refined oils are not necessarily high viscosity index oils since oils of intermediate viscosity index are sometimes produced from quite low viscosity index stocks by a severe refining which causes a substantial reduction in the natural inhibitor content of the oil and thereby produces an oil having a correspondingly reduced stability. From the above it should be apparent that over-refined oils are not limited to those produced by solvent extraction. Other refining processes, e. g. sulfuric acid treatment to produce white oils, remove naturally-occurring inhibitors originally in the oil when the treatment is sufficiently severe and thereby produce over-refinement with the attendant difficulties herein discussed.

In general, over-refined oils may be characterized as having natural inhibitors removed to the point where the corrosiveness of the oil is greater than about 40 mgs. on a 1" x 2" coarse-grained copper-lead bearing in a 72-hour corrosion test (subsequently described in more detail) run

30 under the following conditions:

|             |                                                     |
|-------------|-----------------------------------------------------|
| Air rate    | 30 liters per hour                                  |
| Temperature | 300° F.                                             |
| Catalyst    | 10 gms. of steel wool and<br>a 6" x 1" copper strip |

35 In the appended claims the foregoing 40 mgs. loss in the 72-hour corrosion test is designated as a corrosion index of 40.

The solvent refined oils referred to above, and especially the over-refined oils, are not the only type of oils which become definitely corrosive to the newer bearing metals under normal but severe conditions of use in internal combustion engines. It has been found that a corresponding 45 adverse reaction, namely, corrosion of alloy bearing metals such as cadmium-silver alloys, also occurs in paraffinic base oils which have not been solvent refined or over refined. These corrosion difficulties sometimes cause bearing failure after 50 only a few thousand miles of operation. The higher the viscosity index of the lubricating oil the more pronounced in general is the tendency

to corrosion of the kind referred to above. Generally speaking, the problem is encountered in oils having viscosity indexes of 75 and higher, and becomes of major magnitude in oils having a viscosity index of 80 to 85 or higher.

Thirdly, the newer engines require that the crankcase lubricants operate under significantly higher temperatures than heretofore required. It is found that lubricating oils, which are satisfactory and non-corrosive on newer alloy bearings at lower temperatures heretofore normally encountered, become unduly corrosive to these same bearings at the higher temperatures. These higher temperatures approach the borderline of stability of organic compounds and relatively small increases in temperature therefore magnify many-fold the difficulties of inhibiting corrosion and other deterioration such as formation of "varnish," carbon, or sludge.

This invention provides a corrosion inhibitor capable of reducing to a very low level, even at temperatures of 325° F. or above, the corrosive tendencies of hydrocarbon oils which become corrosive during use (though initially non-corrosive), such as highly paraffinic and/or over-refined hydrocarbon lubricating oils.

Problems in lubrication of internal combustion engines have been further multiplied by the necessity for addition of stabilizers capable of inhibiting the deterioration of the lubricating oil at elevated temperatures. As engine conditions became more severe, piston ring sticking, "varnish" formation on pistons and cylinder walls, and deposition of hard carbon on the piston wall above the top piston ring, have caused trouble in engine operation. These particular difficulties are met by incorporation of stabilizing agents such as aryl metal oxides (metal phenates), salts of aryl carboxylic acids, salts of polycarboxylic acids which preferably have been partially esterified, salts of alkyl carboxylic acids containing a polar group (e. g. mercapto, thio-keto, thioether, amino, cyano, phosphino, oxy-keto, and hydroxy groups, and the like) near a carboxyl group of the acid, and metal alcoholates. These types of stabilizers are relatively non-corrosive and some have a corrosion inhibiting function under less severe lubricating conditions.

In naphthenic base lubricating oils, or even in oils of intermediate refinement and intermediate viscosity index (e. g. a viscosity index of less than 75) which are not over-refined, various corrosion inhibitors are highly effective under severe service. However, when an over-refined or high viscosity index oil (e. g. of 80 viscosity index or more) is used as a base stock and when the oil is to do service under extreme conditions on corrosion-sensitive alloy bearings, the difficulties presented have seemed almost insurmountable. Thus there was presented a combination of circumstances not previously encountered, namely: (a) the necessity for lubricating corrosion-sensitive hard alloy bearings, (b) the desirability of using a base oil stock inherently more corrosive to such bearings than lower viscosity index or less highly refined oils, and (c) more severe operating conditions, as respects temperature and speed, than the lubricating engineer had previously been requested to meet.

Under this new combination of circumstances it was found that the above-mentioned non-corrosive stabilizers against deterioration at elevated temperatures catalyzed corrosion by the oil although these compounds remained non-

corrosive in themselves. Also, it was discovered that various corrosion inhibitors found to be effective to prevent corrosion even by the over-refined or higher viscosity index stocks in the absence of the stabilizers were not effective as anti-catalysts to destroy the catalytic corrosion of the stabilizers in such oils. In other words, the anti-catalytic action of an inhibitor in un-compounded hydrocarbon oils formed no adequate basis for predicting that the same inhibitor would selectively "poison" the stabilizing agent of compounded oils and destroy the agent's catalysis of corrosion without also destroying its catalytic stabilizing action against deterioration at elevated temperatures.

A feature of this invention comprises the provision of a lubricating oil containing a new combination of additives. This new combination of additives is highly effective, both as respects stabilization against deposition of adhesive or resinous materials at elevated temperatures and prevention of corrosion of alloy bearings, when incorporated in over-refined lubricating oils and oils having a viscosity index higher than 75, e. g. a viscosity index of 80 to 85 or higher. Since the new combination of additives is effective even in hydrocarbon lubricating oils which are relatively non-responsive to corrosion inhibitors and stabilizers, the combinations disclosed in more detail hereinafter are exceedingly powerful additives for more responsive oils, such as naphthenic or mixed base lubricants containing naturally-occurring inhibitors in normal quantities or in oils having a viscosity index of less than 80.

35 The corrosion inhibitors of this invention comprise long carbon chain multi-bridged thioalkyl compounds having carbon-to-carbon chains of twenty or more carbon atoms in length, and the preferred type is termed herein "paraffin wax polythio-dimers."

36 The term "dimer" as used herein designates a type of product such as produced by linking together two molecules of hydrocarbon structure by a condensation reaction. Such a reaction is 45 illustrated by condensation of a chlorinated hydrocarbon with an inorganic sulfide whereby a chlorine atom from each of two molecules is displaced and a divalent sulfur atom takes up the free valence of each molecule to thereby 50 connect the molecule together, thus:



55 The carbon chains so condensed need not be identical or of the same number of carbon atoms to fall within the meaning of the term "dimer" as used herein. Similarly, the term "trimer" is used to designate compounds in which three 60 molecules are connected by such a condensation reaction, and the term "thiomer" is generic to dimers and trimers in which sulfur is the bridging link. Thiomers of a liquid consistency, even though very viscous at ordinary atmospheric 65 temperatures, are preferred and mixtures which are predominantly dimers or trimers yield the best results. The term "multi-bridged" as applied to these compounds requires that there be more than one sulfur bridge between at least 70 one pair of the condensing molecules.

The term "paraffin wax polythio-dimer" designates a condensation product of two molecules of hydrocarbon structure in which at least two sulfur atoms independently connect alkyl carbon chains containing at least twenty carbon

atoms. Such a dimer is produced by a condensation of two polyhalogenated alkyl molecules containing at least twenty carbon atoms and in which at least two halogen atoms are split out from each alkyl molecule and at least two sulfur atoms replace the free valences of the two molecules.

Modifications within the scope of the invention in its broader aspects include multi-bridged thio compounds in which the terminal valences of the sulfur bridges are separated by two or more intervening carbon atoms of the chain. At least one long carbon chain should be present in the compounds. By "long carbon chain" it is intended to designate a carbon chain having twenty or more carbon atoms. Relatively straight chains are preferred, although branching in the chain is not precluded; for example, butene and isobutene polymers yield long carbon chains having some branches but are suitable for the purposes of this invention. Paraffin wax is an illustration of a composition containing long carbon chains of outstanding value for synthesis of the corrosion inhibitors herein disclosed.

The corrosion inhibiting thiomers of this invention may contain organic or inorganic substituents in one or more of the carbon chains. Examples of such substituents are the halogens, chlorine, bromine and iodine, ester groups, hydroxyl groups, and metal carboxylate groups.

The corrosion inhibitors of this invention may be prepared by various methods. The following are equations for exemplary reactions:

(1) Reaction of halogenated long chain hydrocarbons and an inorganic sulfide in the presence of added sulfur:



(2) Preparation of a mercaptide and reaction with a halogenated hydrocarbon, one or both being long chain compounds:



(3) Oxidation of polymercaptan or polymercaptide with various oxidizing agents:



It has been discovered that a reaction product comprising an unknown mixture of thiomers is an outstanding corrosion inhibitor. This reaction product contains a mixture of different sulfides which cooperate in some unknown manner to produce a powerful corrosive inhibiting action effective at high temperatures and in high viscosity index oils. The reaction product is believed to be a mixture of multi-bridged thiomers, monothio ethers, dithio ethers, and probably a small proportion of trithio ethers. This particular reaction product is one of applicants' preferred species. The reaction product is herein designated "paraffin wax thiomers" and comprises the product of the reaction of a halogenated paraffin wax (preferably containing from about 15 to about 25% chlorine) and an inorganic sulfide such as sodium sulfide or polysulfide.

In order to illustrate the invention and facilitate the practice thereof by those skilled in the art, the following examples of methods of preparing wax thiomers are given:

#### PREPARATION OF CHLORINATED WAX

Crude white scale wax is melted and heated to about 150° to 200° F. and chlorine gas is passed through the melt. The temperature is preferably kept between these limits by adjusting the rates of heating and inflow of chlorine. The density of the mix increases rapidly as the chlorination proceeds and the gravity of the reaction product is thus a measure of the degree of chlorination. When the chlorine content of the wax has reached a desirable percentage the flow of chlorine gas is cut off and the mixture is blown with either nitrogen or air until substantially free of either chlorine gas or hydrogen chloride. The chlorinated wax is a straw-colored liquid which slowly darkens on standing. Exemplary inspections of such chlorinated waxes are as follows:

| Batch  | Per cent Cl | Gravity, °A.P.I. |
|--------|-------------|------------------|
| 1..... | 27.5        | 9.0              |
| 2..... | 28.1        | 8.9              |

#### PREPARATION OF WAX THIOMERS

Utilizing a chlorinated wax such as the above, the wax thiomers may be prepared as follows:

## EXAMPLE 1

The proportions of the reactants are given in the table below:

| Reactants                                 | Grams  | Gram moles |
|-------------------------------------------|--------|------------|
| Chlorinated wax (27.5% chlorine)          | 8,520  | 19         |
| Sodium sulfide (60-62% Na <sub>2</sub> S) | 3,760  | 20.5       |
| Sulfur                                    | 693    | 21.7       |
| Alcohol                                   | 19,000 | 414        |
| Water                                     | 3,185  | 176        |

1 23,000 cc.

The sodium sulfide utilized was approximately a trihydrate and the amount of water added was just sufficient to produce Na<sub>2</sub>S·9H<sub>2</sub>O.

In preparing the wax thiomers the chlorinated wax and alcohol are first thoroughly mixed in a vessel equipped with a stirrer and a reflux condenser. The sodium sulfide is dissolved in the heated water. The sulfur is added and the mixture boiled and stirred until the sulfur dissolves in the aqueous solution. This aqueous solution is added to the alcoholic solution of the chlorinated wax and the whole is refluxed at 185° F. (atmospheric pressure) for twenty hours. The reaction product is then washed with water until free of alcohol and inorganic salts and then dried by air-blowing it at elevated temperature. After drying, the final product is filtered.

In a preferred embodiment of the invention the reaction is carried out under conditions such that substantially all the chlorine in the chlorinated wax is removed. In order to facilitate production of this type of product it is preferred that the chlorinated wax contain only about 16% chlorine.

The following table gives analytical results on the various batches of paraffin wax thiomers prepared with some variations in the method of operation:

| Method <sup>1</sup> | Vis. at 100° | Percent S | Molecular weight |
|---------------------|--------------|-----------|------------------|
| 1                   | 1,825        | 12.0      | 724              |
| 2                   | 3,313        | 13.6      | 690              |
| 1                   | 1,740        | 11.1      | 500              |
| 2                   | 1,685        | 12.0      | 827              |
| 1                   | 1,711        | 11.8      | 650              |
| 1                   | 1,680        | 11.4      | 753              |
| 1                   | 1,867        | 11.5      | 703              |
| 1                   | 1,922        | 11.6      | 746              |
| 1                   | 1,677        | 11.2      | 750              |
| 1                   | 1,998        | 10.4      | 697              |
| 2                   | 2,003        | 11.6      | —                |

<sup>1</sup> Method 1—Both alcohol and water are used as in the description given above. Method 2—Only alcohol is used as a solvent, and the sodium sulfide and sulfur are added directly to the chlorinated wax in alcohol. Method 3—Half the quantity of alcohol and water are used.

## EXAMPLE 2

To insure a wax thiomer substantially free of chlorine the following process was utilized:

Chlorinated wax in this example contained 16% chlorine and anhydrous sodium sulfide was used. No water was added and the alcohol was anhydrous. The proportions were as follows:

| Reactants                      | Grams | Gram moles |
|--------------------------------|-------|------------|
| Chlorinated wax (16% chlorine) | 800   | 1.9        |
| Sodium metal                   | 100   | 4.35       |
| Alcohol (100%)                 | 1,600 | 35         |
| Sulfur                         | 69.4  | 2.16       |

The sodium was dissolved in 800 grams of alcohol and half of the resulting sodium ethylate solution saturated with hydrogen sulfide to yield anhydrous sodium hydrosulfide. To this solution the

other half of the sodium ethylate was added. The chlorinated wax was dissolved in 800 grams of alcohol and heated to 160° F. The alcoholic reaction product of sodium ethylate and sodium hydrogen sulfide (anhydrous sodium sulfide) was added and the sulfur stirred in. The whole mixture was refluxed for nineteen hours, washed, dissolved in ethyl ether and dried with anhydrous sodium sulfate. After filtering, the ether was evaporated off.

|                      |       |      |
|----------------------|-------|------|
| Yield                | grams | 701  |
| Viscosity at 100° F. | —     | 1224 |
| Percent S            | —     | 12.6 |
| Percent Cl           | —     | 1.8  |

## EXAMPLE 3

According to this method wax multi-bridged mono-thio-dimers may be prepared as follows:

Chlorinated wax (15 to 25% chlorine) was reacted with an alcoholic solution of sodium hydroxide to yield wax mercaptan by the reaction—



The wax mercaptan is then converted to alkali metal mercaptides by reaction with caustic soda or sodium ethylate as follows:



The wax mercaptide is then reacted with additional chlorinated wax (15 to 25% chlorine) in alcoholic solution to give a wax multi-bridged sulfide—



A typical product of this method had a molecular weight of 873, a sulfur content of 6.8%, and a chlorine content of 2.2%.

The proportions of the corrosion inhibitors disclosed herein may vary from about 0.1% to about 2% by weight based on the oil. In the less corrosive and more stable oils 0.25% is sufficient, while in more corrosive and less stable oils 1% or more may be necessary. The lighter grades of lubricating oils require somewhat more compounding. In an oil such as a solvent refined S. A. E. 30 lubricant from Kettleman Fields, California crude, 0.25% of the corrosion inhibitor has been found sufficient even in the presence of other stabilizers such as metal phenates.

In general, it has been found that the corrosion inhibitors of this invention are outstanding and not the mere equivalent of the various other sulfides. For example, the same corrosion inhibiting action in over-refined or high viscosity index lubricating oils is not obtainable with ordinary thioethers or disulfides of the type formulae—



respectively. The multi-bridged sulfur structures give a corrosion inhibiting action, particularly in over-refined oils or oils having a viscosity index greater than 75, under conditions where various other thioethers and disulfides of the conventional structure are not fully satisfactory. For example, an S. A. E. 10 lubricating oil from a certain Colombian crude is a particularly diffi-

cult oil to adequately stabilize against corrosion. In such an oil, a monothioether of the type—



is not equivalent to paraffin thiomers as shown 5 by the following data:

| Oil                                                                                                        | Test 1, 325° F., strip corrosion test—mg. wt. loss, fine grained Cu-Pb, 72 hours | Test 2, 300° F., strip corrosion test—mg. wt. loss, coarse grained Cu-Pb, 72 hours | Test 3, bearing corr. test in high speed Diesel engine—mg. wt. loss per full connecting rod |          |
|------------------------------------------------------------------------------------------------------------|----------------------------------------------------------------------------------|------------------------------------------------------------------------------------|---------------------------------------------------------------------------------------------|----------|
|                                                                                                            |                                                                                  |                                                                                    | 68 hrs.                                                                                     | 246 hrs. |
| Colombian S. A. E. 10+0.5% sulfurized metal phenate+0.25% metal organo-phosphate+1.0% cetyl ethyl sulfide  | 26.0                                                                             |                                                                                    | 55                                                                                          | 1 204    |
| Colombian S. A. E. 10+0.5% sulfurized metal phenate+0.25% metal organo-phosphate+1.5% cetyl ethyl sulfide  | 12.2                                                                             | 88.2                                                                               | 40                                                                                          | 1 150    |
| Colombian S. A. E. 10+0.5% sulfurized metal phenate+0.25% metal organo-phosphate+1% paraffin wax thiomeric | 8.6                                                                              | 24.9                                                                               | 9.5                                                                                         | 31       |

<sup>1</sup> By extrapolation.

Likewise, a disulfide of the type formula—



is not the equivalent of a paraffin wax thiomeric having substantially the same sulfur content. This is illustrated by the following data:

| Oil                                                                                                                                    | Test 2, 300° F., strip corrosion test—mg. wt. loss, coarse grained Cu-Pb, 72 hours | Test 3, bearing corr. test in high speed Diesel engine—mg. wt. loss per full connecting rod |          |
|----------------------------------------------------------------------------------------------------------------------------------------|------------------------------------------------------------------------------------|---------------------------------------------------------------------------------------------|----------|
|                                                                                                                                        |                                                                                    | 68 hrs.                                                                                     | 246 hrs. |
| Colombian S. A. E. 10+0.5% sulfurized metal phenate+0.25% metal organo-phosphate+1.0% paraffin wax thiomeric (11.8% sulfur)            | 25                                                                                 |                                                                                             |          |
| Colombian S. A. E. 10+0.5% sulfurized metal phenate+0.25% metal organo-phosphate+1.0% disulfide (R-S-S-R <sub>1</sub> ) (12.3% sulfur) | 85                                                                                 |                                                                                             |          |

From these data it is evident that the paraffin wax thiomeric is from four to eight times as effective as cetyl ethyl sulfide, and over three times as effective as a conventional dialkyl disulfide structure with about the same sulfur content in the inhibiting agent. The limit established by the Caterpillar Tractor Company in the high speed Diesel engine corrosion test is 50 mg. in 246 hours for oils of "exceptional quality." The above data show that paraffin wax thiomers are capable of producing an oil meeting the test for exceptional quality, whereas the other sulfides, although highly effective as corrosion inhibiting agents, do not yield an oil of exceptional quality with Colombian base stocks. As stated above, it should be borne in mind that this Colombian base stock is very difficult to handle from the corrosion standpoint, and this particular type of oil was selected for the above tests in order to emphasize the exceptional properties of the corrosion inhibiting agents herein disclosed.

The strip corrosion data above given were obtained in corrosion tests carried out in the following manner: Glass tubes two inches in diameter and twenty inches long were immersed in an oil bath, the temperature of which was automatically controlled to within  $\pm 1^{\circ}$  F. of the test temperature indicated. Approximately 300 cc. of oil under test was placed in each tube and air was bubbled through it. Strips of the different types of the bearing metals were placed in the oil. The weight loss of each strip was recorded. Before 70 weighing, each strip was washed in petroleum ether and carefully wiped with a soft cotton cloth. The duration of the test was 72 hours. The loss in weight in milligrams in the foregoing corrosion test is termed the corrosion index of the oil.

In test 1 the temperature was 325° F. as indicated. Ten liters of air per hour were bubbled through the test oil and a copper catalyst was utilized.

5 In test 2 the temperature was 300° F. as indicated. 30 liters of air per hour were bubbled

through the test oil and both a copper strip and 10 grams of steel wool were placed in the oil as catalysts. The bearing metal subjected to corrosion in test 2 was a strip of coarse grained copper-lead bearing. This second type test is the one designated previously for characterizing over-refined oils.

30 Test 3 is carried out in a high speed Diesel engine by operation under the following conditions:

|                      |          |
|----------------------|----------|
| R. P. M.             | 1400     |
| Brake horsepower     | 32       |
| Jacket temperature   | 200 ° F. |
| Oil sump temperature | 210 do   |
| Air to radiator      | 125 do   |
| Oil change           | hours 60 |

35 The corrosion inhibitors of this invention need not be single pure compounds. As a practical matter, the thiomers are usually mixtures of different compounds. When all of the carbon chains in the thiomers are long the mixtures contain dimers predominantly with smaller proportions of higher homologues such as trimers or even tetramers. As the number of long chain molecules in the thiomers is increased, viscosity also increases and oil solubility decreases until a point is reached where normally solid substantially oil-insoluble products are obtained. It is 50 possible to obtain oil dispersions of the solid products but a liquid viscous readily oil-soluble thiomeric is preferred.

40 Reference has been made in the foregoing specification to the effectiveness of the inhibitors of this invention for selectively "poisoning" certain stabilizers to minimize the catalytic action thereof on corrosion without destroying the desired catalytic action of such additives in stabilizing the lubricating oil against deterioration at elevated temperatures. Types of stabilizing agents 55 previously mentioned are aryl metal oxides (metal phenates), salts of aryl carboxylic acids, salts of polycarboxylic acids which preferably have been partially esterified, salts of alkyl carboxylic acids containing a polar group near a carboxyl group of the acid, and metal alcoholates.

60 Incorporation of the multi-bridged thioalkyl compounds heretofore disclosed in hydrocarbon oils having a viscosity index greater than 75 or over-refined oils enhances the responsiveness of these oils to the immediately foregoing types of stabilizers. Thus the multi-bridged thioalkyl compounds act as sensitizers in high viscosity 65 index or over-refined hydrocarbon oils for sta-

bilizing agents of the anti-piston-ring-sticking type. The corrosion inhibitors herein disclosed are accordingly multi-functional and are therefore both a sensitizer and an inhibitor of corrosion.

The corrosion inhibitors hereinbefore disclosed cooperate with aryl metal oxides to give a superior oil. Examples of aryl metal oxides are polyvalent metal salts of phenols of the type formula—



in which  $u$ ,  $v$ ,  $w$ ,  $x$  and  $y$  are selected from the group consisting of hydrogen or radicals of hydrocarbon structure. The phenol preferably contains at least one alkyl group having more than four carbon atoms. The term "radicals of hydrocarbon structure" is intended to include alkyl, aryl, aralkyl, alkaryl or cyclic nonbenzenoid groups which may or may not contain inorganic constituents. Likewise, this term includes radicals which contain hydroxyl groups, ether, thioether, keto, thioketo or carboxyl groups.

The aryl metal oxides also may be metal salts of polynuclear phenols, e. g. salts of polyamyl naphtholates.

Examples of specific aryl metal oxides are alkaline earth metal salts of phenols containing a decyl, dodecyl, tetradecyl, cetyl, octadecyl, eicosyl or wax substituent; aluminum salts of phenols containing a decyl, dodecyl, tetradecyl, cetyl, octadecyl, eicosyl or wax substituent; magnesium salts of phenols containing a decyl, dodecyl, tetradecyl, cetyl, octadecyl, eicosyl or wax substituent; and similar salts of alkyl substituted polyhydroxy phenols. Other metals, e. g. tin, zinc, cadmium, chromium, iron, cobalt and nickel, may be substituted for the foregoing metals.

These compounds may be prepared by methods disclosed in the art.

The following data exemplify the effectiveness of the corrosion inhibitors herein disclosed in reducing the corrosivity of lubricants containing aryl metal oxides:

| Oil                                                                                       | 300° F. corr. test—mg. wt. loss, coarse grained copper-lead |         |         |
|-------------------------------------------------------------------------------------------|-------------------------------------------------------------|---------|---------|
|                                                                                           | 24 hrs.                                                     | 48 hrs. | 72 hrs. |
| Colombian S. A. E. 10 (VI=77)-----                                                        | 24.7                                                        | 55.8    | 105.8   |
| Colombian S. A. E. 10 (VI=77) + 0.5% calcium cetyl phenate-----                           | 129.1                                                       | 180.2   | 191.4   |
| Colombian S. A. E. 10 (VI=77) + 0.5% calcium cetyl phenate + 1% paraffin wax thiomer----- | 8.0                                                         | 25.4    | 33.5    |

Sulfurized metal phenates are particularly useful in combination with the multi-bridged sulfur corrosion inhibitors herein disclosed. The sulfurized metal phenates may be formed by reaction of the foregoing aryl metal oxides, particularly polyvalent metal salts of mononuclear phenols, with a small amount of sulfur. About  $\frac{1}{8}$  to  $1\frac{1}{2}$  gram atoms of sulfur per mol of metal phenate may be utilized in carrying out the sulfurization reaction. Preferably, the weight of sulfur is equivalent to about  $\frac{1}{2}$  to 1 gram atom per mol of the phenate. The reaction of the sulfur and metal phenate is desirably carried out in an organic solution. For example, the metal phenate may be dissolved in a small amount of

5 a hydrocarbon oil to form a concentrated solution of 50% by weight or more of the phenate in the oil. The preferred proportion of sulfur is then added to this solution, the reacting ingredients stirred and heated at 300° to 320° F. for about one hour, or until substantially complete reaction is obtained as indicated by the fact that a copper strip will show only a reddish-purple coloring after five minutes' submersion in the reaction mixture at 300° F.

10 Examples of aryl metal oxides which may be sulfurized are calcium, barium, strontium, magnesium, zinc, cadmium, aluminum, tin, chromium, iron, cobalt and nickel aryl metal oxides.

15 The corrosion inhibitors of this invention also cooperate with aryl metal oxides containing aryl sulfide substituents to yield a superior oil. Examples of such aryl metal oxides are illustrated by the following type formulae:



20 45 where  $R$  and  $R_1$  are radicals of hydrocarbon structure, and  $M$  is a metal, preferably a polyvalent metal such as calcium, barium, strontium, magnesium, aluminum, zinc, tin and chromium.

50 55 The effectiveness of the corrosion inhibitors of this invention in combination with the above type sulfide substituted aryl metal oxides is shown by the following data:

| Oil                                                                                                         | 325° F., strip corr. test—mg. wt. loss |         |         |
|-------------------------------------------------------------------------------------------------------------|----------------------------------------|---------|---------|
|                                                                                                             | 24 hrs.                                | 48 hrs. | 72 hrs. |
| Solvent refined oil base S. A. E. 30 (VI=88) + 0.75% metal phenate disulfide-----                           | 17.2                                   | 27.3    | 32.1    |
| Solvent refined oil base S. A. E. 30 (VI=88) + 0.75% metal phenate disulfide + 1% paraffin wax thiomer----- | 1.5                                    | 3.7     | 6.4     |
| Standard Diol HD (VI=37)-----                                                                               | 29.3                                   | 89.4    | 112.2   |
| Standard Diol HD (VI=37) + 1% paraffin wax thiomer-----                                                     | 12.3                                   | 15.1    | 16.1    |

65 70 An oil solution of a metal phenate containing an aryl sulfide group and of the type listed in the foregoing table may be obtained under the trade-name "Paranox 56," a product of Standard Oil Company of New Jersey. 2½% of the Paranox 56 may be added to the oil to obtain 0.75% by weight based on the oil of the metal phenate containing an aryl sulfide substituent. The Standard Diol HD referred to in the above table is an oil sold under that brand name by Standard

Oil Company of New Jersey and believed to contain a small amount of a compound of the type formula—



where R is an alkyl radical, M is an alkaline earth metal, and  $x$  is 1 or 2. In any event the paraffin wax thiomer is operative both with the type of compounds mentioned and in the compounded commercial oils indicated.

Salts of aryl carboxylic acids and the corrosion inhibitors disclosed herein may be utilized in combination to give a superior lubricant. Salts of this type are exemplified by the following type formulae:



where R is a radical of hydrocarbon structure; M is a metal, e. g. calcium, barium, strontium, magnesium, cadmium, zinc, aluminum, tin, chromium, iron, cobalt or nickel; and X is a substituent such as  $-\text{NH}_2$ ,  $-\text{NR}_2$ ,  $-\text{OH}$ ,  $-\text{Cl}$ ,  $-\text{Br}$ ,  $-\text{I}$ ,  $-\text{NO}_2$ ,  $-\text{OM}$ ,  $-\text{SH}$ ,  $-\text{CN}$ ,  $-\text{OCN}$ ,  $-\text{SCN}$ , and the like.

The effectiveness of this combination is illustrated by the following data:

| Oil                                                                                                         | 325° F., strip corr. test—<br>mg. wt. loss |         |         |
|-------------------------------------------------------------------------------------------------------------|--------------------------------------------|---------|---------|
|                                                                                                             | 24 hrs.                                    | 48 hrs. | 72 hrs. |
| Kettleman (Calif.) S. A. E. 30 (VI=86) + 0.5% calcium polyamyl naphthoyl benzoate                           | 50.7                                       | 154.9   | 179.5   |
| Kettleman (Calif.) S. A. E. 30 (VI=86) + 0.5% calcium polyamyl naphthoyl benzoate + 1% paraffin wax thicmer | 11.9                                       | 12.3    | 12.3    |
| Socony-Vacuum RD8-203 (VI=64)                                                                               | 28.7                                       | 75.7    | 107.1   |
| Socony-Vacuum RD8-203 (VI=64) + 1% paraffin wax thicmer                                                     | 24.5                                       | 48.7    | 52.3    |

The calcium polyamyl naphthoyl benzoate referred to in the above table is a compound of the type formula—



The Socony-Vacuum RD8-203 is an oil believed to contain a small amount of a tin salt of a paraffin wax substituted salicylic acid. In any event, the paraffin wax thiomers is operative with such salts and in the compounded oils of this name.

Salts of polycarboxylic acids in combination with the corrosion inhibitors disclosed herein may

be utilized to yield superior lubricants. Exemplary type formulae of polycarboxylic acids from which these salts may be formed are as follows:



10 in which  $n$  may be zero or a whole number, generally from 1 to 8 inclusive,  $x$  is a whole number from 1 to  $n$ , and in which there may or may not be alkyl, aryl, aralkyl or carbocyclic substitution to increase oil solubility. Improved salts of this type are obtained when  $n$  is greater than 1 and the acid contains a polar group substitution in a position alpha, beta, gamma, delta or epsilon to the carbon atom of the salt-forming carboxylic acid group. The term "polar group" as used herein includes the following:

Metallo-carboxyl,  $-\text{COOM}$   
 Hydroxyl,  $-\text{OH}$   
 Amino,  $-\text{NH}_2$   
 Oxy,  $-\text{OR}$   
 Metallo-oxy,  $-\text{OM}$   
 Keto,  $=\text{O}$   
 Thioketo,  $=\text{S}$   
 Mercapto,  $-\text{SH}$   
 Cyano,  $-\text{CN}$   
 Cyanate,  $-\text{OCN}$   
 Thiocyanate,  $-\text{SCN}$

and the like.

The effectiveness of this combination is illustrated by the following data:

| Oil                                                                                                  | 325° F., strip corr. test,<br>mg. wt. loss |         |         |
|------------------------------------------------------------------------------------------------------|--------------------------------------------|---------|---------|
|                                                                                                      | 24 hrs.                                    | 48 hrs. | 72 hrs. |
| 40                                                                                                   |                                            |         |         |
| Kettleman (Calif.) S. A. E. 30 (VI=86) +<br>0.5% calcium cetyl citrate                               | 2.5                                        | 3.5     | 4.3     |
| Kettleman (Calif.) S. A. E. 30 (VI=86) +<br>0.5% calcium cetyl citrate + 1% paraffin<br>wax thiomer. | 0.8                                        | 2.6     | 3.8     |

Calcium, barium, strontium, magnesium, zinc, cadmium, aluminum, tin, chromium, iron, cobalt and nickel salts of the polycarboxylic acids, preferably partially esterified, may be utilized. Examples of acids from which such salts may be prepared by known methods are: oxalic acid, malonic acid, isosuccinic acid, gluteric acid, adipic acid, pimelic acid, suberic acid, sebatic acid, fumaric acid, maleic acid, malic acid, tartronic acid, tartaric acid, citric acid, aminosuccinic acid and the like. It is preferred that each of the above acids be partially esterified and that the metal salts be a salt of a partially esterified acid.

Examples of salts of alkyl carboxylic acids containing a polar group near a carboxyl group of the acid are: the calcium, barium, strontium, magnesium, zinc, tin, aluminum, chromium, iron, cobalt and nickel salts of alpha, beta or gamma hydroxy lauric, myristic, palmitic, stearic and arachidic acids; the calcium, barium, strontium, magnesium, zinc, tin, aluminum, chromium, iron, cobalt and nickel salts of alpha, beta or gamma thio, mercapto, mercaptide or thiono substituted lauric, myristic, palmitic, stearic and arachidic acids; and the calcium, barium, strontium, magnesium, zinc, tin, aluminum, chromium, iron, cobalt and nickel salts of alpha, beta or gamma amino substituted lauric, myristic, palmitic, stearic and arachidic acids. The effectiveness of these salts in lubricating oils may be enhanced

by use in combination with the multi-bridged thioalkyl compounds herein disclosed.

Examples of metal alcoholates which may be added to hydrocarbon oils together with the multi-bridged thioalkyl inhibitors comprise the alkali, alkaline earth, aluminum, and heavy metal alcoholates, e. g. sodium, potassium, calcium, barium, strontium, magnesium, zinc, cadmium, tin, aluminum, chromium, iron, cobalt and nickel alcoholates. Examples of alcohols utilized to form the metal alcoholates are the higher alcohols, such as amyl, hexyl, heptyl, octyl, nonyl, decyl, dodecyl, tetradecyl, hexadecyl, octadecyl, ceryl, myricyl and unsaturated alcohols, such as are derived from lanolin.

For the purposes of clarity and emphasis it is again pointed out that each of the multi-bridged thioalkyl compounds, and particularly the paraffin wax thiomers hereinbefore disclosed, may be utilized either as a corrosion inhibitor or as a sensitizer for hydrocarbon oils to be stabilized with any of the aryl metal oxides, salts of aryl carboxylic acids, salts of polycarboxylic acids, salts of alkyl carboxylic acids containing a polar group, and the metal alcoholates above disclosed. In some instances, as for example in over-refined or high viscosity index oils having a viscosity index greater than 75, the principal function of the thiomers may be that of a sensitizer rather than a corrosion inhibitor. In other instances, as when the hydrocarbon oil being stabilized is only moderately refined or has a viscosity index less than 75 and the service to be encountered by the compounded oil is severe or with corrosion-sensitive bearings, the principal function of the thiomers may be that of a corrosion inhibitor. In still other situations the thiomers may serve as multi-functional agents to both inhibit corrosion and sensitize the base oil to stabilization with the salt-type inhibitor.

The proportion of the salt-like inhibitors, that is, of the aryl metal oxides, salts of aryl carboxylic acids, salts of polycarboxylic acids, salts of alkyl carboxylic acids containing a polar group, and the metal alcoholates above disclosed, may vary from about 0.1% to 2% by weight in the finished oil. From approximately .5% to 1.5% is usually preferred.

Another aspect of this invention comprises the provision of an activator for the multi-bridged thioalkyl compounds disclosed herein. These activators enhance the effectiveness of the thiomers herein disclosed in a manner which has not been explained and is not understood. The activators preferably comprise either an acid ester, that is, a partially esterified acid of a strong acid-forming element such as phosphorus, or of a weak acid-forming element such as arsenic, antimony or boron, or a salt of acids of these strong or weak acid elements containing an organic substituent. Either the acid ester alone, or the salt alone, or mixtures of salts and acid esters of any of the foregoing may be used as an activator. These types of activators, when utilized in combination with the foregoing multi-bridged thioalkyl compounds, enhance the corrosion inhibiting or sensitizing action thereof. This is true even though the activator may not, when added alone, be a sensitizing agent for the oil being stabilized.

Illustrative activators which may be added to hydrocarbon oils, such as mineral lubricating oil, according to this invention comprise metal salts in which the metals are selected from groups II, III, IV and VI of Mendelyeef's Table of the

Elements. Specific examples of such metals are: calcium, barium, strontium, magnesium, zinc, tin, cadmium, aluminum, chromium, iron, cobalt and nickel. Likewise, the alkali metal and ammonium salts are not precluded.

The salts of substituted acids of phosphorus utilized as activators and illustrating the derivatives of strong acid-forming elements are preferably formed from substituted oxyacids of pentavalent phosphorus of the following type formula:



where R may be alkyl, aryl, alkaryl, aralkyl or cyclic nonbenzenoid radicals. Substituted phosphoric acids containing at least twelve carbon atoms are preferred, but where the salts are sufficiently soluble in oil, acids containing fewer carbon atoms may be utilized. Examples of preferred type acids are alkyl and alkaryl substituted phosphoric acids having at least twelve carbon atoms in the molecule. It is to be understood that the broader aspects of the invention include salts of other types of acids of phosphorus containing more than twelve carbon atoms. Additional examples of such substituted oxyacids of phosphorus are as follows:



Phosphonic acid



Monoester of phosphonic acid



Phosphinic acid

where R and R<sub>1</sub> may be alkyl, aryl, alkaryl, aralkyl or cyclic nonbenzenoid groups which, in turn, may be pure hydrocarbon constituents or oxygenated hydrocarbons such as alcohols, ketones, esters and ethers, or hydrocarbons containing substituents such as halogens (chlorine, bromine, iodine), amino, or nitro groups. Likewise, R and R<sub>1</sub> may be an oil-soluble heterocyclic constituent; for example, a radical containing a nitrogen ring.

In general, salts of substituted derivatives of acids of phosphorus, such as phosphorous acid, H<sub>3</sub>PO<sub>3</sub>; hypophosphoric acid, H<sub>2</sub>PO<sub>3</sub>; orthophosphoric acid, H<sub>3</sub>PO<sub>4</sub>, pyrophosphoric acid, H<sub>4</sub>P<sub>2</sub>O<sub>7</sub>, and the sulfur analogues of these acids fall within the broadest aspects of the invention. By "acids of phosphorus containing an organic substituent" or by "substituted acids of phosphorus" wherever used herein it is intended to designate acids of phosphorus containing an organic group of the types previously listed. The organic groups may be either directly attached to the phosphorus atom of the compound or attached thereto through an intervening atom, such as oxygen or sulfur. The term "oxyacids of phosphorus" is used to designate throughout the specification and claims acids of phosphorus in which only an oxygen atom may intervene be-

tween the hydrogen and phosphorus atoms of the parent acid.

Additional examples of activators comprising derivatives of weak acid-forming elements are metal salts or acid esters derived from acids selected from the following groups: 5

**TYPE 1.—ACIDS OF BORON CONTAINING AN ORGANIC SUBSTITUENT**



Diesters of dithio-organo boric acid



Diesters of dithio-organo thio-boric acid

**TYPE 2.—ACIDS OF ARSENIC CONTAINING AN ORGANIC SUBSTITUENT**

**A.—Trivalent arsenic**



Organic ortho-arsinous acid (arsine dihydroxides)



Organic arsenous acid (diorgano substituted arsenic hydroxide)



Monoester of organo ortho-arsinous acid



Organic monothio-arsinous acid



Organic dithio-arsinous acid



Monothio-ester of organo arsenous acid



Monoester of organo monothio-arsinous acid



Monoester of organo dithio-arsinous acid



Monoester of arsenous acid



Diesters of arsenous acid



Monothio-ester of arsenous acid

|                                                                                                                                                             |    |                                                                                                                                    |
|-------------------------------------------------------------------------------------------------------------------------------------------------------------|----|------------------------------------------------------------------------------------------------------------------------------------|
| <br>Monothio-ester of monothio-arsenous acid                                | 5  | <br>Monoester of thion-monothiol-arsenic acid    |
| <br>Monoester of trithio-arsenous acid (monoester of dithio-arsenous acid) | 10 | <br>Organo monothiol-arsenic acid               |
| <br>Monoester of trithio-arsenous acid (monoester of dithio-arsenous acid) | 15 | <br>Organo dithiol-arsenic acid                 |
| <br>Monothio-diester of arsenous acid                                      | 20 | <br>Monothio-ester of organo arsenic acid       |
| <br>Dithio-diester of arsenous acid                                        | 25 | <br>Monothio-ester of organo thiol-arsenic acid |
| <br>Monothio-diester of monothio-arsenous acid                             | 30 | <br>Diorgano substituted thion-arsinic acid     |
| <b>B.—Pentavalent arsenic</b><br><br>Organo arsenic acid                   | 35 | <br>Diorgano substituted dithio-arsinic acid    |
| <br>Disubstituted organo arsenic acid                                      | 40 | <br>Monoester of arsenic acid                   |
| <br>Monoester of organo arsenic acid                                     | 45 | <br>Diorgano substituted thiol-arsinic acid   |
| <br>Organo thion-arsenic acid                                            | 50 | <br>Monoester of arsenic acid                 |
| <br>Organo thion-monothiol-arsenic acid                                  | 55 | <br>Diester of arsenic acid                   |
| <br>Organo trithio-arsenic acid                                          | 60 | <br>Monothio-ester of arsenic acid            |
| <br>Monoester of organo thion-arsenic acid                               | 65 | <br>Monothio-ester of monothiol-arsenic acid  |
| <br>Monothio-ester of organo thion-arsenic acid                          | 70 | <br>Monoester of dithiol-arsenic acid         |
| <br>Monoester of organo trithio-arsenic acid                             | 75 |                                                                                                                                    |



Monothio-diester of arsenic acid



Dithio-diester of arsenic acid



Monothio-diester of monothiol-arsenic acid



Monoester of monothiol-arsenic acid



Diester of monothiol-arsenic acid



Monothio-ester of monothiol-arsenic acid



Monothio-ester of thion-monothiol-arsenic acid



Monothio-ester of tetrathio-arsenic acid



Monothio-diester of thion-arsenic acid



Dithio-diester of thion-arsenic acid



Monothio-diester of thion-monothiol-arsenic acid



In all of the foregoing type formulae R and R' are radicals of hydrocarbon structure. It is understood that by the term "hydrocarbon structure" it is intended to include hydrocarbon groups containing polar radicals such as OH, SH, Cl, NH<sub>2</sub> and COOH. Likewise, this term includes radicals containing ether, sulfide and ester groups.

It should be borne in mind that in the foregoing type formulae all of the acids listed may not exist as such and that it is the esters or salt-like derivatives thereof with which the present invention is concerned. Accordingly, existence of the free acid in a stable form is not a prerequisite to the preparation of the derivatives thereof contemplated herein. It should also be observed that various of the salt-like derivatives

are relatively insoluble in organic solvents such as hydrocarbon oils. However, oil-solubility is not an absolute prerequisite for utility of the present invention in its broadest aspects, as will be explained in more detail hereinafter; nevertheless, oil-soluble compounds are preferred. Some of the salt-like compounds and esters are unstable at high temperatures. When the compounded oil is to encounter high temperature conditions during use compounds known or found to be more stable at elevated temperatures should be selected.

Activating agents contemplated within the broader aspects of the invention are in general salts, and preferably polyvalent metal salts, of the following acid reacting compounds: organic substituted derivatives of acids of boron, such as orthoboric, H<sub>3</sub>BO<sub>3</sub>; mesoboric, H<sub>4</sub>BO<sub>5</sub>; metaboric, H<sub>2</sub>B<sub>2</sub>O<sub>4</sub>; dihydrotiboric, H<sub>4</sub>BO<sub>6</sub>; hexahydrotetraboric, H<sub>8</sub>BO<sub>9</sub> (once called pyroboric acid); dihydrotetraboric, H<sub>2</sub>B<sub>4</sub>O<sub>7</sub>; hexahydrohexaboric, H<sub>8</sub>B<sub>6</sub>O<sub>12</sub>; dihydrohexaboric, H<sub>2</sub>B<sub>6</sub>O<sub>10</sub>; hexahydro-octoboric, H<sub>8</sub>B<sub>8</sub>O<sub>15</sub>; dihydro-octoboric, H<sub>2</sub>B<sub>8</sub>O<sub>13</sub>; dihydrodecaboric, H<sub>2</sub>B<sub>10</sub>O<sub>16</sub>; dihydrododecaboric, H<sub>2</sub>B<sub>12</sub>O<sub>19</sub>; organic substituted derivatives of acids of arsenic, such as alkyl arsine hydroxides or oxides, alkyl arsine sulfides, dialkyl arsine hydroxides or oxides, dialkyl arsine sulfides, aryl arsine hydroxides or oxides, alkaryl arsine hydroxides or oxides, aryl or alkaryl arsine sulfides and sesquisulfides, diaryl arsine hydroxides or oxides, dialkaryl arsine hydroxides or oxides, diaryl or dialkaryl arsine sulfides, alkyl arsionic acids, alkyl arsine disulfides, alkyl arsinic acids, aryl arsionic acids, aryl di-arsionic acids, halogenated aryl arsionic acids, nitroaryl arsionic acids, amino aryl arsionic acids, hydroxy aryl arsionic acids, carboxy aryl arsionic acids, alkaryl arsionic acids, alkaryl diarsionic acids, halogenated alkaryl arsionic acids, aryl arsinic acids, alkaryl arsinic acids, aryl trithio-arsionic acids, alkaryl trithio-arsionic acids, aryl arsine disulfides, and alkaryl arsine disulfides.

The proportion of activating agents herein disclosed which may be added according to the principles of the present invention may vary depending upon the uses involved and the properties desired. As little as 0.05% by weight of various of the compounds gives measurable improvements. From approximately 0.1% to 2% of the compounds may be added to liquid lubricants. In general, from approximately 0.25% to 0.75% has been found preferable, particularly when used in conjunction with from approximately 0.25% to 1% of an aryl metal oxide and 0.5% to 1.5% of the paraffin wax thiomers.

A preferred embodiment of this invention provides a mineral oil composition containing three types of components, namely:

- (1) A metal salt of an organic acid in an amount sufficient to inhibit deterioration of the oil. This type of stabilizing agent has been previously disclosed herein in detail and examples given of aryl metal oxides, salts of aryl carboxylic acids, salts of polycarboxylic acids which preferably have been partially esterified, salts of alkyl carboxylic acids containing a polar group near a carboxyl group of the acid, and metal alcoholates. These salts, as hereinbefore disclosed, may be used in this preferred embodiment;

- (2) A corrosion inhibitor and/or a sensitizer in an amount sufficient substantially to reduce corrosion and/or enhance the responsiveness of the hydrocarbon oil to the stabilizing action of the metal salt stabilizer. When the base oil being stabilized is of high viscosity index or over-refined, this second ingredient usually functions primarily as a sensitizer. When the base oil is of low viscosity index or low refinement, the ingredient may serve primarily as a corrosion inhibitor. In moderately refined or moderate viscosity index base oils, this type of ingredient serves both as a sensitizer and a corrosion inhibitor. The corrosion inhibitor and/or sensitizer is a long carbon chain multi-bridged thioalkyl compound of the type previously disclosed herein. The many examples given in this specification may be utilized in the present preferred embodiment of the invention but, as previously indicated, the paraffin wax thiomers are outstanding.
- (3) An activator for the sensitizer and/or corrosion inhibitor for increasing the effectiveness thereof. The activators comprise either an acid ester, that is, a partially esterified acid of phosphorus, arsenic, antimony or boron, or a salt of acids of these elements containing an organic substituent, as disclosed hereinbefore.

The following data on oils compounded with the above three types of ingredients are illustrative:

The strip corrosion tests in Tables I and II were carried out in the same manner as described previously for 325° F. and 300° F. corrosion tests, respectively.

- 5 In the compounded oils containing the combination of three additives as above described, the proportions may be as previously indicated, namely, from about 0.1% to 2% by weight, and preferably from approximately 0.5% to 1.5% by weight based on the oil, of the salts of organic acids; from about 0.1% to about 2% by weight based on the oil of a corrosion inhibitor and/or sensitizer, and preferably from about 0.25% to 1.5% thereof; and from as little as 0.05% to 2% by weight based on the oil of the activator, from approximately 0.25% to 0.75% being preferable.
- 10 The compounded hydrocarbon oils herein disclosed may have one or more advantages depending upon the particular compounding agent or combination of compounding agents selected, the proportions utilized, and the environment which the lubricating oil is to encounter. It should be observed, for example, that even though a compounded oil may be somewhat corrosive to one particular type of bearing alloy, other bearings may be little if at all affected by such corrosive action. Hence, compounding agents or combinations thereof which may not be particularly desirable for lubrication of a special type of bearing, where corrosion becomes a factor of importance, may nevertheless be highly useful and extremely advantageous in conjunction with the operation of internal combustion engines
- 15 20 25 30 35 having corrosive-resistant bearing metals. Like-

TABLE I

325° F. strip corrosion test on S. A. E. 30 oil from Kettleman crude (California) + 0.5% sulfurized calcium cetyl phenate + 0.25% calcium cetyl phosphate + 0.25% thiomer

| Vis. at 100° F. | Mol. wt. | Multi-bridged thiomer compounding agent |            |                         |                       |                                                              | Preparation by— | Cu-Pb wt. loss mmg. |             |            | Viscosity increase at 210° F. | Neut. No. | Naphtha insoluble |  |  |
|-----------------|----------|-----------------------------------------|------------|-------------------------|-----------------------|--------------------------------------------------------------|-----------------|---------------------|-------------|------------|-------------------------------|-----------|-------------------|--|--|
|                 |          | Percent S                               | Percent Cl | Percent Cl in orig. wax | Percent by wt. in oil | 24 hrs. 48 hrs. 72 hrs.                                      |                 |                     |             |            |                               |           |                   |  |  |
|                 |          |                                         |            |                         |                       | 24 hrs.                                                      | 48 hrs.         | 72 hrs.             | 24 hrs.     | 48 hrs.    | 72 hrs.                       |           |                   |  |  |
| 1,753           | 680      | 12.2                                    | 11.5       | 26                      | 0.25                  | Reaction of chlorinated paraffin wax with sodium sulfide.    | 11.0<br>0.7     | 30.5<br>1.7         | 44.0<br>4.4 | 7.6<br>4.4 | 1.28<br>0.83                  | 45<br>1   |                   |  |  |
| 3,031           | 936      | 13.3                                    | 10.3       | 26                      | 0.25                  | do                                                           | +0.3<br>3.6     | 0.0<br>11.0         | 1.4<br>14.2 | 7.6<br>7.8 | 0.46<br>1.94                  | 2<br>16   |                   |  |  |
| 1,012           | 504      | 7.5                                     | 3.7        | 15.4                    | 0.25                  | Reaction of chlorinated lubricating oil with sodium sulfide. | 6.3             | 16.7                | 19.1        | 7.1        | 1.15                          | 10        |                   |  |  |
| 590             | 873      | 6.8                                     | 2.2        | 16                      | 0.25                  | Reaction wax polymercaptide with chlorinated wax.            |                 |                     |             |            |                               |           |                   |  |  |

TABLE II

300° F. strip corrosion test (coarse grained bearings) on S. A. E. 10 oil from Colombian crude + 0.5% sulfurized calcium cetyl phenate + 0.25% calcium cetyl phosphate + 1% thiomer

| Vis. at 100° F. | Mol. wt. | Multi-bridged thiomer compounding agent |            |                         |                       |                                                                            | Preparation by— | Cu-Pb wt. loss mmg. |               |            | Viscosity increase at 210° F. | Neut. No. | Naphtha insoluble |  |  |
|-----------------|----------|-----------------------------------------|------------|-------------------------|-----------------------|----------------------------------------------------------------------------|-----------------|---------------------|---------------|------------|-------------------------------|-----------|-------------------|--|--|
|                 |          | Percent S                               | Percent Cl | Percent Cl in orig. wax | Percent by wt. in oil | 24 hrs. 48 hrs. 72 hrs.                                                    |                 |                     |               |            |                               |           |                   |  |  |
|                 |          |                                         |            |                         |                       | 24 hrs.                                                                    | 48 hrs.         | 72 hrs.             | 24 hrs.       | 48 hrs.    | 72 hrs.                       |           |                   |  |  |
| 1,753           | 680      | 12.2                                    | 11.5       | 26                      | 0.1                   | Reaction of chlorinated paraffin wax with sodium sulfide.                  | 0.4<br>0.4      | 112.4<br>9.8        | 259.4<br>29.6 | 3.4<br>2.5 | 4.18<br>1.57                  | 71<br>27  |                   |  |  |
| 1,561           | 550      | 11.1                                    | 12.6       | 26                      | 1                     | Reaction of chlorinated paraffin wax with sodium sulfide (iron present).   | 3.7             | 17.8                | 34.4          | 2.0        | 1.32                          | 27        |                   |  |  |
| 1,224           | 1,525    | 12.6                                    | 1.7        | 16                      | 1                     | Reaction of chlorinated paraffin wax with sodium sulfide.                  | 0.2             | 6.7                 | 12.6          | 1.9        | 1.30                          | 18        |                   |  |  |
| 2,886           | 1,500    | 18.0                                    | 1.0        | 16                      | 1                     | Reaction of chlorinated paraffin wax with sodium sulfide (+ extra sulfur). | +3.1            | +3.2                | +3.7          | 1.5        | 0.84                          | 17        |                   |  |  |
| 1,012           | 504      | 7.5                                     | 3.7        | 15.4                    | 1                     | Reaction of chlorinated lubricating oil with sodium sulfide.               | 3.7             | 22.1                | 65.9          | 2.1        | 2.19                          | 25        |                   |  |  |
| 590             | 873      | 6.8                                     | 2.2        | 16                      | 2                     | Reaction wax polymercaptide with chlorinated wax.                          | 2.0             | 15.6                | 29.6          | 2.6        | 1.43                          | 24        |                   |  |  |

wise, combinations of compounding agents which are not sufficiently powerful to stabilize a particular oil stock under the most extreme conditions may, nonetheless, be highly advantageous in such oils where the environment to be encountered is not so severe. The present invention in its broader aspects is therefore not limited to the particular compounding agent or combination of ingredients giving the greatest stability or passing all of the very severe tests which have been devised. The invention embraces various of the less advantageous additives or combinations thereof which may find utility in particular applications where all possible improvements in properties of the oil may not be required or where the standard of performance may not be so high.

The compounding agents and combinations of this invention appear at present to find their greatest utility in over-refined or highly paraffinic mineral lubricating oil stocks, which stocks have heretofore been the most difficult to stabilize. However, it is to be understood that the invention is not limited to such base stocks since advantages herein disclosed may be obtained with moderately refined or less paraffinic lubricating oils or even low viscosity index lubricants.

The compounded hydrocarbon oils of this invention may be utilized as turbine oils, cable oils, electric switch oils, transformer oils and the like, as well as in crankcase lubricants for internal combustion engines and especially Diesel engines. The compounding agents of this invention may also be added to hydrocarbon oils containing additional ingredients, such as pour point depressants, oiliness agents, extreme pressure addition agents, blooming agents, compounds for enhancing the viscosity index of the hydrocarbon oil, thickening agents and/or metal soaps in grease-forming proportions or in amounts insufficient to form grease, as in the case of mineral castor machine oils or other compounded liquid lubricants.

In the foregoing disclosure an upper limit of approximately 2% by weight based on the oil of each of the compounding agents has been indicated as sufficient for a finished oil. The present invention also embraces solutions containing more than 2% of the novel combination of compounding agents. Concentrates containing high percentages of the additives of this invention comprise a convenient method of handling the compounding agents, and the concentrated solutions may be sold and used as addition agents for lubricants in general. Thus mineral oil solutions containing as much as 50% or more by weight of the compounding agents may be prepared. Such concentrated solutions are adapted for dilution with hydrocarbon lubricating oil to yield a finished product containing, for example, from approximately 0.5% to 1.5% by weight of a metal phenate; from approximately 0.25% to 1.5% by weight of a paraffin wax thiomer; and from approximately 0.25% to 0.75% by weight based on the oil of a metal salt of an acid of phosphorus containing an organic substituent. Concentrated solutions of the additives in organic solvents capable of dilution with mineral lubricating oil to form a homogeneous mixture containing the above proportions of compounding agents comprise a part of this invention.

While the character of the invention has been described in detail and numerous examples of the compounds given, this has been done by way

of illustration only and with the intention that no limitation should be imposed upon the invention thereby. It will be apparent to those skilled in the art that numerous modifications and variations of the illustrative examples may be effected in the practice of the invention which is of the scope of the claims appended hereto.

We claim:

1. A lubricating oil having a corrosion index greater than about 40 containing a paraffin wax thiomer in an amount sufficient to inhibit the corrosive action of said lubricating oil.
2. A lubricating oil having a corrosion index greater than about 40 containing a paraffin wax poly-(monothio)dimer in an amount sufficient to inhibit the corrosive action of said lubricating oil.
3. A lubricating oil having a corrosion index greater than about 40 containing a paraffin wax di-(monothio)dimer in an amount sufficient to inhibit the corrosive action of said lubricating oil.
4. A viscous hydrocarbon oil subject to deterioration at elevated temperature, an aryl metal oxide in an amount sufficient substantially to inhibit said deterioration, and an inhibitor capable of reducing catalysis of corrosion by said aryl metal oxide without destroying the stabilizing action thereof, said inhibitor comprising a paraffin wax thiomer.
5. A viscous hydrocarbon oil subject to deterioration at elevated temperature, a metal salt of an aryl carboxylic acid in an amount sufficient substantially to inhibit said deterioration, and an inhibitor capable of reducing catalysis of corrosion by said salt of an aryl carboxylic acid without destroying the stabilizing action thereof, said inhibitor comprising a paraffin wax thiomer.
6. A viscous hydrocarbon oil subject to deterioration at elevated temperature, a metal salt of a partially esterified polycarboxylic acid in an amount sufficient substantially to inhibit said deterioration, and an inhibitor capable of reducing catalysis of corrosion by said salt of a partially esterified polycarboxylic acid without destroying the stabilizing action thereof, said inhibitor comprising a paraffin wax thiomer.
7. A viscous hydrocarbon oil subject to deterioration at elevated temperature, a metal alcoholate in an amount sufficient substantially to inhibit said deterioration, and an inhibitor capable of reducing catalysis of corrosion by said metal alcoholate without destroying the stabilizing action thereof, said inhibitor comprising a paraffin wax thiomer.
8. A lubricant comprising a viscous hydrocarbon oil subject to deterioration at elevated temperature, a metal salt of an organic acid in an amount sufficient substantially to inhibit said deterioration, a paraffin wax thiomer sensitizer for the hydrocarbon oil capable of enhancing its responsiveness to the stabilizing action of said metal salt, and an activator capable of enhancing the effectiveness of said thiomer sensitizer, said activator comprising a salt of an acid of phosphorus containing an organic substituent.
9. A lubricant comprising a viscous hydrocarbon oil subject to deterioration at elevated temperature, an aryl metal oxide in an amount sufficient substantially to inhibit said deterioration, a paraffin wax thiomer sensitizer for the hydrocarbon oil capable of enhancing its responsiveness to the stabilizing action of said aryl metal oxide, and an activator capable of enhancing the effec-

tiveness of said thiomer sensitizer, said activator comprising a salt of an acid of phosphorus containing an organic substituent.

10. A lubricant comprising a viscous hydrocarbon oil subject to deterioration at elevated temperature, a metal salt of an aryl carboxylic acid in an amount sufficient substantially to inhibit said deterioration, a paraffin wax thiomer sensitizer for the hydrocarbon oil capable of enhancing its responsiveness to the stabilizing action of said salt of an aryl carboxylic acid, and an activator capable of enhancing the effectiveness of said thiomer sensitizer, said activator comprising a salt of an acid of phosphorus containing an organic substituent.

11. A lubricant comprising a viscous hydrocarbon oil subject to deterioration at elevated temperature, a metal salt of a partially esterified polycarboxylic acid in an amount sufficient substantially to inhibit said deterioration, a paraffin wax thiomer sensitizer for the hydrocarbon oil capable of enhancing its responsiveness to the stabilizing action of said salt of a partially esterified polycarboxylic acid, and an activator capable of enhancing the effectiveness of said thiomer sensitizer, said activator comprising a salt of an acid of phosphorus containing an organic substituent.

12. A lubricant comprising a viscous hydrocarbon oil subject to deterioration at elevated temperature, a metal alcoholate in an amount sufficient substantially to inhibit said deterioration, a paraffin wax thiomer sensitizer for the hydrocarbon oil capable of enhancing its responsiveness to the stabilizing action of said metal alcoholate, and an activator capable of enhancing the effectiveness of said thiomer sensitizer, said activator comprising a salt of an acid of phosphorus containing an organic substituent.

13. A lubricant comprising a viscous hydrocarbon oil, an inhibitor comprising a paraffin wax thiomer, and an activator for enhancing the effectiveness of said inhibitor comprising a salt of an organo-substituted acid of an element selected from the group consisting of phosphorus, boron and arsenic.

14. A lubricant comprising a viscous hydrocarbon oil, an inhibitor comprising a paraffin wax thiomer, and an activator for enhancing the effectiveness of said inhibitor comprising a salt of an acid of phosphorus containing an organic substituent.

15. A lubricant comprising a hydrocarbon lubricating oil, from approximately 0.1% to 2% by weight based on the oil of an aryl metal oxide of a polyvalent metal, from approximately 0.1% to approximately 2% by weight based on the oil of a paraffin wax thiomer, and from approximately 0.05% to 2% by weight based on the oil of a polyvalent metal salt of an acid of phosphorus containing an organic substituent.

10. A lubricant comprising a hydrocarbon lubricating oil, from approximately 0.1% to 2% by weight based on the oil of a polyvalent metal salt of an aryl carboxylic acid, from approximately 0.1% to approximately 2% by weight based on the oil of a paraffin wax thiomer, and from approximately 0.05% to 2% by weight based on the oil of a polyvalent metal salt of an acid of phosphorus containing an organic substituent.

15. A lubricant comprising a hydrocarbon lubricating oil, from approximately 0.1% to 2% by weight based on the oil of a polyvalent metal salt of a partially esterified polycarboxylic acid, from approximately 0.1% to approximately 2% by weight based on the oil of a paraffin wax thiomer, and from approximately 0.05% to 2% by weight based on the oil of a polyvalent metal salt of an acid of phosphorus containing an organic substituent.

17. A lubricant comprising a hydrocarbon lubricating oil, from approximately 0.1% to 2% by weight based on the oil of a polyvalent metal salt of a partially esterified polycarboxylic acid, from approximately 0.1% to approximately 2% by weight based on the oil of a paraffin wax thiomer, and from approximately 0.05% to 2% by weight based on the oil of a polyvalent metal salt of an acid of phosphorus containing an organic substituent.

18. A viscous hydrocarbon oil having a corrosion index greater than about 40, containing a paraffin wax thiomer having a long chain containing at least 20 carbon atoms, said paraffin wax thiomer being present in a small amount sufficient substantially to reduce the corrosion index of said oil and to sensitize said oil to the stabilizing action of an aryl metal oxide.

19. A viscous hydrocarbon oil having a corrosion index greater than about 40 and a paraffin wax thiomer sensitizer for the hydrocarbon oil, said sensitizer having a long chain containing at least 20 carbon atoms and being present in a small amount sufficient to enhance the stabilizing action of an aryl metal oxide on said hydrocarbon oil, and an activator capable of enhancing the effectiveness of said paraffin wax thiomer sensitizer, said activator comprising a polyvalent metal salt of an organo-inorganic acid.

BRUCE B. FARRINGTON.  
VICTOR M. KOSTAINSEK.  
GEORGE H. DENISON, JR.